

# UNITED STATES PATENT OFFICE.

ALEXANDER McLENNAN, OF ROSS, ENGLAND.

## PROCESS FOR THE TREATMENT OF LEATHER WITH INDIA RUBBER.

1,425,530.

Specification of Letters Patent. Patented Aug. 15, 1922.

No Drawing.

Application filed January 21, 1922. Serial No. 530,978.

To all whom it may concern:

Be it known that I, ALEXANDER McLENNAN, a subject of the King of Great Britain, residing in Ross, Herefordshire, England, have invented certain new and useful Improvements in Processes for the Treatment of Leather with India Rubber, of which the following is a specification.

This invention relates to the treatment of leather with india rubber and it refers more particularly to a process such as forms the subject of United States Letters Patent granted to me under No. 970,734.

The present invention has for its object certain improvements primarily designed to secure a more perfect impregnation of the leather with the rubber whereby a greater amount of rubber is forced into the leather, and its vulcanization therein, and further to provide the leather with a better gripping surface, particularly desirable when the leather is employed for the soles of boots, or machinery belting for example.

According to the present invention the leather after having been subjected to any necessary preliminary treatment is treated with a clarifying or grease removing solution formed by dissolving crystalline powdered sulphur in a solvent which may either be carbon bisulphide or tetrachlorethane. The liquid just referred to, which may be termed the stock solution, is allowed to stand for a time with occasional agitation after which the undissolved sulphur is precipitated by the addition, to a predetermined quantity, of the stock liquid, of a solution comprising acetone.

Instead of the above precipitants ether and benzol may be used, alone or in combination with the foregoing.

To the mixture thus formed paraffin oil or petrol is added the resultant liquid being employed for the treatment of the leather for removing the grease therefrom.

The leather is then sprayed with the clarifying solution and preferably this is effected by placing the said leather in a suitable receptacle having a well fitting lid whereby when the leather has been well saturated the receptacle may be closed and evaporation as far as possible prevented. The leather after the treatment just described is left for a certain time when it is removed and allowed to dry.

The leather when dry is buffed upon the flesh side and is placed in a suitable recep-

tacle which may have a steam or hot water jacket, or other means may be provided whereby its contents can be heated. The receptacle just referred to contains a solution of india rubber formed by dissolving rubber in coal tar solvent, naphtha, or benzol, which is thinned to the desired consistency by the addition of heavy grade petroleum spirit and paraffin oil. After remaining in the solution just referred to for a certain time the leather is removed and worked by hand after which it is replaced in the solution and after a certain time is again worked by hand. With leather of a medium weight two workings with a final immersion are usually found sufficient but if found necessary a further treatment or treatments in the manner described may be given.

After its final immersion the leather is removed and any superfluous solution is allowed to drain therefrom.

The leather is then drummed with a rubber solution as just above described but of slightly greater density.

To the solution just referred to there is added, after the drumming operation has been in progress for a certain time, a further solution of slightly greater density than that first referred to composed of the same components as the second solution. During the final period of the drumming there is added at intervals solution containing gutta percha, balata, gum mastic and gum dammar, and finally about 1 hour before the conclusion of the treatment chloride of sulphur solution.

In my above mentioned patent the chloride of sulphur solution was added to the rubber solutions in the tank prior to drumming the leather. This I have found to be detrimental because it had the effect of congealing the solution thereby hindering penetration, unless the solution be kept continually warm, which is difficult and expensive to do, and also because it was found to be injurious to the men working the leather from the tank. In the present instance the chloride or sulphur solution is added in the drum, at the latter end of the treatment when the leather has been thoroughly impregnated with the solutions, the required heat being obtained by the constant revolving of the drum. In this way the desired object is attained, that is avoidance of the injurious effect upon the men and vulcanization of the rubber which has become em-

bedded in the cells of the leather by means of the process.

Whilst it will be understood that I do not desire to limit myself to the precise quantities or proportions stated as it may be found necessary or desirable in practice to vary these according to the condition or characteristics of the leather, temperature, climatic conditions or for other reasons, the following are given as examples which have been

10 found in practice to give very good results when dealing with hides of average weight:

For the stock solution 1 lb. of powdered sulphur was dissolved in about 6 lbs. of carbon bisulphide or tetrachlorethane, the mixture being allowed to stand with occasional agitation for a period of from 6 to 8 hours.

For the precipitating solution:—

20 Ether ----- 18 liquid ozs.  
Acetone ----- 18 liquid ozs.  
Benzol ----- 24 liquid ozs.

which is added to three pints of the stock solution.

25 Assuming that 20 to 30 hides of medium weight are to be treated I have found that good results are obtained if the ingredients are in the following proportions:—

For the first rubber solution 1 lb. of india 30 rubber is dissolved in 1 to  $1\frac{1}{4}$  gallons of coal tar solvent, naphtha or benzol the resultant solution being thinned down with  $1\frac{1}{2}$  to  $1\frac{3}{4}$  gallons of petroleum spirit, preferably heavy grade, and  $1\frac{1}{2}$  to  $1\frac{3}{4}$  gallons paraffin.

35 Or 1 lb. of india rubber dissolved in from  $2\frac{1}{4}$  to  $2\frac{1}{2}$  gallons of coal tar solvent, naphtha or benzol the resultant solution being thinned down with 2 to  $2\frac{1}{4}$  gallons of paraffin.

For the first drumming solution (No. 1) 40 1 lb. of india rubber is dissolved in 1 to  $1\frac{1}{4}$  gallons of coal tar solvent, naphtha or benzol the resultant solution being thinned down with 1 to  $1\frac{1}{4}$  gallons petroleum spirit, preferably heavy grade, and 1 to  $1\frac{1}{4}$  gallons of paraffin.

45 Or 1 lb. of india rubber dissolved in  $1\frac{1}{2}$  to 2 gallons of coal tar solvent, naphtha or benzol the resultant solution being thinned down with  $1\frac{1}{2}$  to  $1\frac{3}{4}$  gallons of paraffin.

50 For the second drumming solution (No. 2) 1 lb. of india rubber is dissolved in 1 to  $1\frac{1}{4}$  gallons of coal tar solvent naphtha, or benzol the resultant solution being thinned down with  $\frac{3}{4}$  to 1 gallons petroleum spirit, preferably heavy grade, and  $\frac{3}{4}$  to 1 gallon paraffin.

55 Or 1 lb. of india rubber dissolved in  $1\frac{1}{2}$  to  $1\frac{3}{4}$  gallons of coal tar solvent naphtha, or benzol, the resultant solution being thinned down with  $1\frac{1}{2}$  to  $1\frac{3}{4}$  gallons paraffin.

For the gutta percha solution 1 lb. of gutta percha is dissolved in a solution formed of 5 to 7 pints of carbon bisulphide or warmed coal tar naphtha or petroleum spirit.

60 65 In the balata solution 1 lb. of balata is dis-

solved in a solution formed of 5 to 7 pints of carbon bisulphide or warmed coal tar naphtha or petroleum spirit.

The gum mastic solution is formed by dissolving 2 lbs. of gum mastic in 2 to 3 pints 70 of benzol or other known solvents.

The gum dammar solution is formed of 2 lbs. of gum dammar dissolved in 4 to 5 pints of benzol or other known solvents.

For the final treatment to one pint of the 75 stock there is added for precipitation purposes 6 liquid ozs. of acetone or any of the other substances before mentioned as being employed as precipitants together with 6 liquid ozs. of ether, 8 liquid ozs. of benzol 80 and 10 to 12 liquid ozs. of chloride of sulphur.

The hides are first drummed for about 6 hours with 12 to 14 gallons, or more according to the number of hides, of the first 85 drumming solution, at the expiration of which 10 to 12 gallons, or more according to the number of hides, of the second drumming solution are introduced and the drumming continued for a further 7 to 8 hours 90 during which period there are introduced at different times the various gum solutions and finally within one hour of the completion of the drumming the chloride of sulphur solution.

95 In practice it is found that when acetone or similar volatile liquids are employed as sulphur precipitants in the formation of the stock solution, particularly where the solution is placed in air-tight glass or other receptacles, it is difficult to keep the stoppers in the said jars when moving them. Under these circumstances it will be found more convenient in the final drumming to place the precipitated stock solution in the drum, the chloride of sulphur being subsequently added, or the chloride of sulphur may be mixed with the stock solution which is then introduced into the drum, or the stock solution may be introduced into the drum and 100 chloride of sulphur immediately thereafter.

Under these circumstances to the final treatment to 3 pints of the stock solution there is added for precipitation purposes 18 liquid ozs. of ether, 18 liquid ozs. of acetone, 115 together with 24 liquid ozs. of Benzol.

110 The same quantity of Chloride of sulphur will be used to each pint of the above mentioned stock solution namely 10 to 12 liquid ozs. but this will be fed into the drum 120 separately from the powdered sulphur solution.

125 It is obvious to one skilled in the art that where, throughout the specification and claims, india rubber is accorded the important place in the formula and process herein, that other soluble vulcanizable gums of similar nature may be substituted for the said india rubber without departing from the spirit or scope of the invention.

## Claims.

1. In a process for impregnating leather with india rubber, drumming the leather in rubber solution; and when the leather is 5 impregnated with the rubber adding to the rubber solution an element for vulcanizing the rubber which has become embedded in the leather.
2. In a process for impregnating leather 10 with india rubber, drumming the leather in a revolving receptacle in rubber solution; and during a final period of the drumming adding to the rubber solution chloride of sulphur solution for vulcanizing the rubber 15 which has become embedded in the leather.
3. In a process for impregnating leather with india rubber, moving the leather in rubber solution in a movable receptacle; and when the leather is impregnated with the 20 rubber, adding to the rubber solution an element for vulcanizing the rubber which has become embedded in the leather; the heat required to prevent congealing of the solution when the vulcanizing element is added being 25 obtained by constant movement of the receptacle.
4. In a process for impregnating leather with india rubber, moving the leather in rubber solution in a moving receptacle; and during a final period of moving the leather 30 adding to the rubber solution chloride of sulphur solution for vulcanizing the rubber which has become embedded in the leather; the heat required to prevent congealing of the solution when the chloride of sulphur 35 solution is added being obtained by constant movement of the receptacle.
5. In a process for impregnating leather with india rubber, treating the leather for impregnating the leather with rubber; and 40 when the leather is impregnated with the rubber treating the leather with an element for vulcanizing the rubber which has become embedded in the leather.

In testimony whereof I have hereunto set 45 my hand in the presence of two witnesses.

ALEXANDER McLENNAN.

## Witnesses:

ERNEST MARTIN BERRY,  
CHARLES WILLIAM PHILLIPS.